

# UNITED STATES PATENT OFFICE.

SILAS R. DIVINE, OF LOCH SHELDRAKE, NEW YORK, ASSIGNOR TO THE  
REND ROCK POWDER COMPANY, OF NEW JERSEY.

## EXPLOSIVE COMPOUND.

SPECIFICATION forming part of Letters Patent No. 289,763, dated December 4, 1883,

Application filed August 8, 1883. (No specimens.)

*To all whom it may concern:*

Be it known that I, SILAS R. DIVINE, of  
Loch Sheldrake, Sullivan county, State of New  
York, and a citizen of the United States, have  
5 invented an Improved Explosive Compound,  
of which the following is a full, clear, and ex-  
act specification.

The object of my invention is to "sensitize"  
or impart increased susceptibility to explo-  
sion to an explosive compound, for use chief-  
ly in blasting, composed of chlorate of pot-  
ash, in a crushed or powdered state, as a solid  
ingredient, and a mixture of nitro-benzole and  
the heavy oil of coal-tar, commonly called  
15 "dead-oil," as a liquid ingredient, so that said  
compound may be readily exploded under var-  
ious conditions of confinement, as in loose or  
"rotten" rock or shale, or in earth, or in the  
open air.

20 My invention consists in an explosive com-  
pound of crushed or powdered chlorate of pot-  
ash, as a solid ingredient therein, and a mix-  
ture of substantially equal parts of nitro-ben-  
zole and dead-oil, as a liquid ingredient there-  
25 in, substantially in the proportions of from  
about four to five parts of said solid to one of  
said liquid ingredient, (as described by me in  
an application for Letters Patent filed July  
23, 1883,) with the wet or moist mass of said  
30 ingredients is united sulphur, in a finely-pow-  
dered state, substantially in the proportions  
hereinafter set forth.

As is stated in said application for Letters  
Patent, above referred to, either perchlorate  
35 or permanganate of potash may be substi-  
tuted for chlorate of potash in the compound,  
and in like manner other liquid nitro com-  
pounds may be substituted for nitro-ben-  
zole, and other fluid hydrocarbons which are  
40 practically non-volatile in a free state at or-  
dinary temperatures—say such as have a  
boiling-point above about 300° Fahrenheit—

may be substituted for the dead-oil; and  
the stated proportions need not, however, be  
strictly adhered to, inasmuch as a preponder- 45  
ance of the nitro-benzole in the mixture con-  
stituting the liquid ingredient will augment  
the strength or power of the explosive, while  
a diminution of the nitro-benzole in said mix-  
ture will decrease such strength or power, and 50  
in the former case it will be found desirable  
to decrease somewhat, and in the latter case  
to increase somewhat, the proportion of the  
chlorate of potash in the compound; and, fur- 55  
thermore, the said solid and liquid ingredi-  
ents may be readily combined by simply al-  
lowing the solid to absorb the liquid.

The proportion in which it is desirable to  
use the sulphur is from about one to three per  
cent. thereof relatively to the mass of the 60  
above-named combined solid and liquid in-  
gredients; but these proportions may be varied  
without departing from the essential feature  
of the invention. The sulphur is united with  
the wet or moist mass of the combined chlo- 65  
rate of potash and liquid ingredient, and this  
may be accomplished by mixing the sulphur  
with the said mass by hand in a suitable ves-  
sel. The danger of spontaneous explosion, at-  
tendant upon mixing sulphur with chlorate of 70  
potash in a dry state, is thus avoided.

What I claim as my invention, and desire  
to secure by Letters Patent, is—

The explosive compound herein described,  
composed of chlorate of potash and a mixture 75  
of nitro-benzole and dead-oil, substantially in  
the proportions stated, with the wet or moist  
mass of which said combined ingredients is  
united sulphur, substantially in the propor-  
tions and as and for the purpose set forth.

SILAS R. DIVINE.

Witnesses:

A. S. FITCH,  
A. G. N. VERMILYA.